

July 9, 1963

W. W. DYRKACZ ET AL

3,097,092

AUSTENITIC ALLOY

Filed July 5, 1961

2 Sheets-Sheet 1



INVENTORS  
Wasil W. Dyrkacz, Clifford R. Hastings  
and Richard K. Pitler

BY

*Robert F. Randig*  
ATTORNEY

July 9, 1963

W. W. DYRKACZ ET AL

3,097,092

AUSTENITIC ALLOY

Filed July 5, 1961

2 Sheets-Sheet 2

| Heat No. | $\chi/\alpha$ | % N | % S  |
|----------|---------------|-----|------|
| 40838    | 2.29          | .28 | .055 |
| 04588    | 3.06          | .45 | .047 |
| 40802    | 2.28          | .23 | .004 |

Fig. 2



*INVENTORS*  
Wasil W. Dyrkacz, Clifford R. Hastings  
and Richard K. Pitler

BY

*Robert T. Bandig*

ATTORNEY

1

3,097,092

**AUSTENITIC ALLOY**

Wasil W. Dyrkacz, Niskayuna, and Clifford R. Hastings, Troy, N.Y., and Richard K. Pitler, Gibsonia, Pa., assignors to Allegheny Ludlum Steel Corporation, Brackenridge, Pa., a corporation of Pennsylvania

Filed July 5, 1961, Ser. No. 121,886  
13 Claims. (Cl. 75—128)

This invention relates to stable, austenitic, age-hardenable alloys suitable for use at temperatures of up to about 1600° F., and in particular to stable, austenitic, age-hardenable alloys which are especially suitable for use as valves and valve components in exhaust systems of internal combustion engines.

The development of new metals and alloys for use as valves and valve components which exhibit high temperature properties superior to those metals and alloys which are commercially available today, has lagged the pace of other similar metallurgical developments because competitive considerations have emphasized valve cost reduction without the sacrifice of physical, chemical and mechanical properties. Thus the supplier who manufactures the metals and alloys from which such valves are made must offer a product which possesses the requisite mechanical properties such as stress-rupture strength and hardness, chemical properties such as corrosion and oxidation resistance, and physical properties such as resistance to thermal fatigue, hot stretching and thermal shock, and at the same time the supplier's product must also exhibit the ability to be fabricated at a minimum cost. These considerations of cost have had their manifestations portrayed in the chemical composition of the metal, the hot workability of the metal, and the machinability of the metal. Thus, with respect to the cost factor as it relates to the chemical composition, it is incumbent upon the metal manufacturer to design his composition so that the costs of raw material alloying components are minimized without the sacrifice of the requisite mechanical, chemical and physical properties necessary in the finished product. In addition, the chemical composition must also be balanced so that the metal will exhibit excellent hot workability, thereby reducing to a minimum all scrap losses which would be incurred during the hot working of the metal from the cast ingot into the semi-finished mill product from which the finished product is manufactured. In the case of valves and valve components, the semi-finished mill product is usually bar stock which must exhibit good upsettability and extrudability over a wide temperature range into a finished valve. Moreover, the semi-finished mill product which the metal manufacturer supplies must also exhibit excellent machinability, especially in the case of valves and valve components, in order to minimize the cost of the finished product. The machinability exhibited by the metal or alloy is integrally related to the chemical composition of the metal or alloy; therefore, the balanced relationship of the alloying components is most critical.

One of the commercially available valve compositions in present use today is an austenitic alloy, referred to hereinafter as Alloy X, which possesses a nominal commercial analysis of about .55% carbon, about 9.5% manganese, low silicon, about 21% chromium, about 4% nickel and about 0.40% nitrogen, about 0.06% sulfur and the balance iron. This composition possesses an acceptable combination of stress-rupture strength, hardness, corrosion and oxidation resistance, resistance to thermal fatigue, hot stretching and thermal shock. However, the designer of the alloy found it to be essential to include about 0.06% sulfur in the composition in order for the alloy to exhibit an economical degree of machinability. However, the machinability was imparted to the alloy at

2

the sacrifice of hot workability, and where the sulfur content exceeded about 0.07% sulfur, high scrap losses resulted in the commercial mill processing of this material. In addition, the over-all effect of the alloying components was such that an extremely narrow range of the sum of the carbon+nitrogen content (0.92% to 0.98%) had to be maintained. Where the sum of the carbon+nitrogen was below this critical range, the finished, heat treated product did not exhibit the requisite hardness. On the other hand, where the sum of the carbon+nitrogen exceeds the upper limit, considerable difficulty is encountered in shearing and machining operations. In addition, where the sum of the carbon+nitrogen exceeds about 0.98%, the alloy is difficult to work in the blooming mill, it being found that a greater number of passes and larger power requirements are necessary, thus adding to the cost of fabricating the alloy. While a higher temperature would rectify the difficulties encountered in the blooming operation, such higher temperature cannot be employed where more than about 0.06% sulfur is present because the alloy becomes hot-short.

Another composition which has found some acceptance in commercial usage today is an alloy referred to herein as Alloy Y and which contains a low carbon content, about 5% nickel, about 5% manganese and about 21% chromium. Criticism of this material has resulted from the fact that the material could not be utilized in manufacturing a one-piece valve. Apparently the carbon content is insufficient for developing the requisite hardness. Therefore, in order to maintain stem and tip wear resistance in valves, it has been found preferable to make the stem and tip of the valve out of a different material.

In order to alleviate these conditions, the alloy of the present invention possesses mechanical properties akin to those exhibited by Alloy X, yet the alloy of the present invention exhibits excellent hot workability and machinability without the necessity of utilizing high sulfur contents, thus obviating any hot workability problems which have been associated with the prior art alloy.

An object of the present invention is to provide an alloy which is suitable for use at elevated temperatures of up to about 1600° F. and which possesses an acceptable combination of mechanical, chemical and physical properties which make said alloy suitable for use as valves and valve components.

Another object of this invention is to provide a stable, austenitic, age-hardenable alloy suitable for use as valves and valve components operating at elevated temperatures of up to about 1600° F., which alloy is characterized by having a balanced chemical composition within narrow limits.

A further object of the present invention is to provide a stable, austenitic, age-hardenable alloy which is suitable for valves and valve components operating at temperatures of up to about 1600° F. and which possess excellent hot workability and machinability through a balanced chemical composition.

A more specific object of the present invention is to provide a stable, austenitic, age-hardenable alloy having a critical balance between the carbon, nitrogen, manganese, nickel, chromium and silicon contents, together with a very narrow range of sulfur content and which possesses excellent hot workability and machinability.

A further specific object of the present invention is to provide a stable, austenitic, age-hardenable alloy suitable for use as valves and valve components suitable for use at temperatures of up to about 1600° F. and which has a critically balanced composition between the austenite formers carbon, nitrogen, manganese and nickel, and the ferrite formers chromium and silicon and which exhibits excellent hot workability and machinability without the

use of excessive amounts of sulfur or other expensive machinability-improving elements.

Other objects of this invention will become apparent when taken in conjunction with the drawings in which:

FIGURE 1 is a graphic illustration of the relative machinability of alloys of both the present invention and prior art alloys, each in the solution heat treated condition, and

FIG. 2 is a graphic illustration of the relative machinability of the alloys of the present invention as well as prior art alloys in the solution treated plus aged condition.

In its broader aspects, the alloy of the present invention contemplates a composition which includes between 0.65% and 0.75% carbon, 5.50% and 6.90% manganese, 0.45% and 0.85% silicon, 20.50% and 22.0% chromium, 1.40% to 1.90% nickel, 0.18% to 0.28% nitrogen, from 0.025% to 0.055% sulfur and the balance iron with incidental impurities. Reference may be had to Table I which illustrates the broad range and the preferred range of composition of the alloy which comes within the scope of the claims which are appended hereto.

TABLE I  
*Chemical Composition*  
[Percent by weight]

| Element | General Range | Optimum Range |
|---------|---------------|---------------|
| C.....  | 0.65-0.75     | 0.68-0.73     |
| Mn..... | 5.50-6.90     | 6.00-6.50     |
| Si..... | 0.45-0.85     | 0.60-0.70     |
| Cr..... | 20.50-22.00   | 21.00-21.50   |
| Ni..... | 1.40-1.90     | 1.60-1.75     |
| N.....  | 0.18-0.28     | 0.20-0.25     |
| S.....  | 0.025-0.055   | 0.025-0.040   |
| Fe..... | Bal.          | Bal.          |

Each of the foregoing elements set forth in Table I performs a vital function in the alloy of the present invention. Carbon is effective for forming austenite which must be controlled within relatively narrow limits in order to insure sufficient hot workability without adversely affecting the machinability of the alloy. In addition, carbon materially contributes to the hardness and strength of the alloy, and it has been found that at least 0.65% carbon is necessary in order to obtain the requisite strength, hardness and a sufficient amount of austenite within the micro-structure of the alloy in order to obtain the optimum combination of hot workability and machinability. Carbon contents in excess of about 0.75% adversely affect the machinability and contribute to reducing the strength and ductility of the alloy. Optimum results appear to be obtained when the carbon content is maintained within the range between about 0.68% and 0.73%. Manganese materially contributes to the austenitic stability of the alloy, and at least 5.50% is necessary. Manganese contents in excess of about 6.9%, while being effective for increasing the austenitic stability, adversely affect the machinability of the alloy because of the higher work-hardening rate imparted by this element. Optimum results appear to be obtained where the manganese content is maintained within the range between 6.00% and 6.50%. Silicon is present within the alloy, and within the range specified materially contributes to the oxidation and corrosion resistance of the alloy. At least 0.45% silicon has been found to be necessary, and silicon contents in excess of about 0.85% appear to adversely affect the mechanical properties of the alloy, especially the stress rupture strength. Silicon is a ferrite-forming element, and as such must be critically balanced against the austenite-forming components as will be more fully explained hereinafter. Optimum results are obtained when the silicon content is maintained within the range between 0.60% and 0.70%.

Chromium is present within the range between 20.50% and 22.0%. Within this range the alloy possesses the required degree of corrosion resistance, especially in atmos-

pheres containing combustion products of leaded fuels. In addition, at least 20.50% chromium is necessary in order to afford the alloy an acceptable measure of resistance to oxidation at elevated temperatures of about 1600° F., and particularly 1100° F. to 1600° F. Chromium contents below about 20.50% result in rapid scaling at hot working temperatures, thereby adversely affecting die life, and thus increasing manufacturing costs. Chromium is also a ferrite former, and as such must be balanced against the austenite formers to insure the proper degree of hot workability without adversely affecting machinability. The most satisfactory combination of properties occurs when the chromium content is within the range between 21.0% and 21.5%. At least 1.40% nickel is used within the alloy of the present invention in that it contributes to the hot strength and hardness of the alloy. However, the nickel content must be maintained at no greater than 1.90%, since increasing the nickel content beyond about 1.90% adversely affects the hardness, the stress rupture strength and the ductility of the alloy.

Nitrogen is highly critical and is present within the alloy as an interstitial hardener. Thus, it has a great influence on the strain hardening rate of the alloy. In addition, nitrogen is a potent austenite-forming element and materially contributes to the strength and stability of the alloy. At least 0.18% nitrogen is necessary within the alloy in order to insure the proper strength and austenite stability. Increasing the nitrogen content to above about 0.28% results in a great increase in the strain hardening rate, adversely affecting the machinability of this alloy, and also increases the resistance to deformation at hot working temperatures, thereby materially increasing fabricating costs. Optimum results appear to be obtained when the nitrogen content is maintained within the range of about 0.20% and 0.25%.

The present alloy also contemplates the presence of sulfur within the composition. At least 0.025% has been found necessary in order to insure the proper degree of machinability within the alloy. Increasing the sulfur content to above about 0.055% does not cause any significant improvement in the machinability, and in addition, sulfur contents in excess of 0.055% seriously limit the hot workability of the alloy, thus causing considerable difficulty in manufacturing the alloy into the semi-finished mill product form. The balance of the alloy comprises substantially all iron, with incidental impurities normally found in the making of such alloys.

The alloy of the present invention is conveniently made in the regular steel mill manner. Substantial success has been realized by making said alloy utilizing the carbon electrode electric arc melting practice to obtain the heat of the desired chemical composition, following which the melt is cast into ingots which are thereafter hot rolled to a convenient semi-finished mill product form, for example, bars. It should be pointed out, however, that other melting practices can be used with equal success, and because of the critically balanced nature of the alloying elements, to be referred to more fully hereinafter, the alloy of the present invention exhibits outstanding hot workability and may be hot worked in any suitable manner on any suitable equipment and is not necessarily limited to hot rolling.

The alloy of the present invention may be used in various forms, and, in this respect, it has been found that the alloy of the present invention is responsive to various heat treatments to obtain a number of desired combinations of properties. In particular, it has been found that the alloy of the present invention may be solution heat treated at a temperature in the range between 1800° F. and 2200° F. for a time period ranging between about 15 minutes and about four hours, followed by a quench. In practice, it has been found that the use of a water quench is quite effective. Subsequently the alloy may be aged at a temperature within the range of about 1200° F. to

about 1700° F. for a time period ranging between about one hour and about 24 hours and thereafter the alloy may be air cooled. When heat treated within the broad temperature range set forth hereinabove, the alloy of the present invention exhibits a good combination of creep rupture properties, hardness and ductility without any adverse effect on the machinability or the corrosion resistance of the alloy.

Where the alloy is to be used in service which requires the highest combination of creep rupture properties and a hardness of  $R_c$  34 minimum, the alloy may be advantageously heat treated by subjecting it to a solution heat treatment at a temperature within the range between 1950° F. and 2200° F. for a time period ranging between 15 minutes and two hours, followed by a rapid cooling to room temperature. Thereafter, the alloy may be aged at a temperature within the range between about 1350° F. and about 1500° F. for a time period ranging between four hours and about 16 hours, followed by air cooling. When thus heat treated, in addition to the alloy's exhibiting the highest combination of creep rupture properties and a minimum hardness of 34  $R_c$ , no adverse effects have been noted in the machinability of the alloy or in the corrosion resistance of the alloy.

Some valve manufacturers prefer to produce a valve which exhibits intermediate creep rupture properties and which may be produced at a low cost without any sacrifice in the corrosion or oxidation resistance nor in the machinability of the alloy. This may be achieved by hot working the alloy into the shape of a valve, solution heat treating the semi-finished valve at a temperature within the range between 1950° F. and 2050° F., followed by a rapid cooling, and thereafter machining the valve shape where necessary to its finish dimensions. The valve in the solution treated condition may then be used directly in an internal combustion engine where it will become aged in use where the valve operates at a temperature within the range between 1100° F. and 1600° F.

Where it is desirable to manufacture the lowest cost valve which possesses adequate creep rupture properties, resistance to oxidation and corrosion and without any adverse effect on the machinability, the alloy may be hot worked, for example, by extruding or forging and upsetting, into the shape of a valve and thereafter the semi-finished valve may be machined to the finished product. As so fabricated, the valve may be used directly in the engine, thus providing the lowest cost valve with adequate properties. Where substantially higher hardnesses are required, the alloy of the present invention is particularly attractive because of the simplified heat treatment which is involved. Once again, the alloy may be either forged or extruded into the shape of a valve, and thereafter the alloy is subjected to a heat treatment at a temperature within the range between 1400° F. to 1700° F. for a time period of up to about eight hours and thereafter the alloy is air cooled. As thus processed, the valve which is formed from the alloy of the present invention will exhibit a hardness of 38  $R_c$  minimum. This hardness is substantially higher than the maximum hardness exhibited by the one-piece austenitic valves in substantially all internal combustion engines which are utilized in passenger cars manufactured today.

When the alloy of the present invention is utilized for valves and valve components, it is desirable that the alloy from which such valves and valve components are made possess mechanical properties which are equivalent to or better than the mechanical properties exhibited by the commercially available alloys in use today. Reference is respectfully directed to Table II which contains a tabulation of the chemical composition of a number of alloys which were made, some of which fall within the scope of the alloy of the present invention, and some of which fall outside the scope of the present invention.

TABLE II  
Chemical Composition  
[Percent by weight]

| Heat No. | C   | Mn  | Si  | Cr   | Ni  | N   | S    | Fe   |
|----------|-----|-----|-----|------|-----|-----|------|------|
| 40839    | .69 | 6.8 | .63 | 20.5 | 1.9 | .29 | .031 | Bal. |
| 40802    | .69 | 6.6 | .72 | 20.6 | 1.9 | .23 | .004 | Bal. |
| A-897    | .51 | 6.3 | .26 | 21.7 | 2.0 | .25 |      | Bal. |
| A-633    | .68 | 6.3 | .58 | 22.0 | 2.1 | .15 |      | Bal. |
| A-901    | .56 | 6.4 | .32 | 22.0 | 2.2 | .22 |      | Bal. |
| A-529    | .61 | 6.4 | .11 | 20.8 | 2.4 | .15 |      | Bal. |
| 40836    | .76 | 6.9 | .23 | 20.6 | 2.3 | .22 | .009 | Bal. |
| 40838    | .70 | 6.2 | .83 | 20.5 | 1.9 | .27 | .055 | Bal. |
| 04588    | .51 | 9.5 | .24 | 21.4 | 3.9 | .44 | .047 | Bal. |
| 04732    | .54 | 9.5 | .11 | 21.3 | 4.0 | .46 | .047 | Bal. |
| 05055    | .69 | 5.8 | .54 | 21.1 | 1.7 | .21 | .031 | Bal. |
| X-1      | .60 | 9.8 | .15 | 20.6 | 3.5 | .45 | .086 | Bal. |
| X-2      | .53 | 9.1 | .19 | 20.6 | 3.5 | .41 | .064 | Bal. |
| B-1      | .66 | 6.1 | .63 | 21.4 | 1.6 | .23 | .021 | Bal. |
| B-2      | .71 | 6.2 | .61 | 21.2 | 1.6 | .24 | .022 | Bal. |
| 8        | .74 | 6.3 | .67 | 21.4 | 2.3 | .24 | .018 | Bal. |

Reference is directed to Table III which contains a comparison of the stress-rupture properties exhibited by one of the presently used commercial alloys referred to as Alloy X and the alloy of the present invention referred to as Alloy B.

TABLE III

## Nominal Stress Rupture Properties

[At temperature 1350° F.]

| Alloy | Stress | Hours to Failure | Percent Elonga- | Percent Red. of Area |
|-------|--------|------------------|-----------------|----------------------|
| X-1   | 20,000 | 175              | 17.7            | 29.9                 |
| X-2   | 20,000 | 249              | 12.0            | 21.0                 |
| X-2   | 20,000 | 307              | 16.5            | 18.9                 |
| B-1   | 20,000 | 617              | 28.0            | 34.0                 |
| B-2   | 20,000 | 647              | 29.0            | 37.0                 |

It will be noted from the test results tabulated in Table III that the alloy of the present invention exhibits outstanding characteristics which are far superior to the mechanical properties exhibited by Alloy X. Alloy B exhibits greater rupture life and is more ductile, as measured by both the percent elongation and percent reduction of area, than Alloy X. Since the test temperature is within the range of operation of exhaust valves of internal combustion engines, the foregoing test results give a realistic appraisal of the use of the alloy for valves and valve components.

In addition to the foregoing stress rupture properties, the alloy of the present invention must also possess sufficient hardness. In this respect, it is customary for the valve manufacturer to specify a minimum hardness of about 34  $R_c$  at room temperature, and a minimum hardness of about 135 BHN at 1400° F. Reference is directed to Table IV which includes a tabulation of the hardness properties and the tensile properties of some of the heats referred to in Table II.

TABLE IV

| Heat No. | BHN |           | Tensile Properties |          |             |              |
|----------|-----|-----------|--------------------|----------|-------------|--------------|
|          | RT  | 1,400° F. | U.T.S.             | .2% Y.S. | Percent El. | Percent R.A. |
| 40837    | 311 | 137       |                    | 70,500   | 32.8        | 30.9         |
| 40839    | 340 | 137       | 154,400            | 95,500   | 36.8        | 35.7         |
| 8        | 302 |           | 146,600            | 79,500   | 3.0         | 4.0          |
| A-897    | 321 |           |                    |          |             |              |
| A-633    | 302 |           |                    |          |             |              |
| A-901    | 311 |           |                    |          |             |              |
| A-529    | 311 |           |                    |          |             |              |

By comparison of the heats listed in Table IV, especially with respect to the nickel content of said heats, it is clear that nickel contents in excess of about 1.90% adversely affect the hardness and ductility of the alloy.

Comparing Heat No. 40839 with Heat No. 8, it is clear that the room temperature hardness is adversely affected. While Heat No. 8 has a yield strength comparable to Heat No. 40837 and a slightly lower tensile strength than Heat No. 40839, it is clear that the ductility of the alloy is seriously affected. Thus it is clear that the nickel content of the present alloy must be limited to a nickel content between 1.40% and 1.90% in order to obtain the requisite hardness and ductility without adversely affecting the stability and machinability of the alloy.

Heretofore it has been stated that the alloy of the present invention is particularly suitable for use as valves and valve components, and through various heat treatments and/or fabrication procedures it is possible to obtain a wide variety of mechanical properties. Reference is directed to Table V which shows the results of hardness measurements conducted on Heat No. 05055, the chemical analysis of which is set forth in Table II, for aging treatments at various temperatures and for various periods of time, the alloy being in the hot worked or in the hot worked plus solution heat treated condition.

TABLE V

[Heat No. 05055]

| Heat Treatment  | Hot Worked,<br>$R_c$ Ave. | Hot Worked<br>+2,150° F.—<br>1 Hr.—W.Q.,<br>$R_c$ Ave. |
|-----------------|---------------------------|--------------------------------------------------------|
| 1,400° F.—4 hr. | 38.9                      | 37.2                                                   |
| 1,400° F.—8 hr. | 39.4                      | 37.9                                                   |
| 1,500° F.—4 hr. | 38.4                      | 37.5                                                   |
| 1,500° F.—8 hr. | 39.4                      | 35.3                                                   |
| 1,600° F.—4 hr. | 39.3                      | 35.3                                                   |
| 1,600° F.—8 hr. | 39.7                      | 34.4                                                   |
| 1,700° F.—4 hr. | 40.2                      | 35.9                                                   |
| 1,700° F.—8 hr. | 39.7                      | 34.4                                                   |

From the data tabulated in Table V, it is clear that the alloy of the present invention responds to a simple aging treatment after the alloy has been hot worked. As thus processed, it is clear from the data set forth in Table V that an aging heat treatment at a temperature within the range between 1400° F. and 1700° F. for various periods of time of up to eight hours is effective for obtaining at least 38  $R_c$  hardness in the alloy. This outstanding hardness is obtained, together with adequate creep rupture properties and without any sacrifice in the corrosion and oxidation resistance nor in the machinability of the alloy. The test results recorded in Table V also illustrate that the alloy of the present invention develops a minimum hardness of  $R_c$  34 where the alloy after hot working is subjected to a solution heat treatment at a temperature of 2150° F. followed by aging at a temperature within the range between 1400° F. and 1700° F. for various time periods of up to about eight hours. As thus processed, the alloy also possesses excellent creep rupture properties and the corrosion and oxidation resistance and machinability are not impaired. Thus the alloy of the present invention is ideally suited for use in valves and valve components.

As was stated hereinbefore, the alloy of the present invention is an age-hardenable, stable, austenitic alloy which contains a critical balance of the chemical composition, and especially the nitrogen and sulfur contents. While the excellent hot workability exhibited by the alloy of the present invention is a significant factor in the overall cost reduction resulting from lower scrap losses and higher yields in fabricating the material from the ingot form to the semi-finished mill product, the most significant cost factor is realized from the excellent machinability of the alloy having a composition within the specific analysis range. These cost reductions are realized from the superior machining qualities of the alloy of the present invention resulting from increased production rates, less down-time for tool change, and a significantly longer tool life. Based on comparative machinability tests con-

ducted under strict laboratory control, the machinability of these alloys was determined to be critically dependent upon the balance of the austenite and ferrite-forming elements, the sulfur content and the nitrogen content, all of which are interrelated. Since the chemical analysis of the material has an extremely profound effect upon its machinability, the presence of the alloying elements within the range set forth hereinbefore in Table I is further characterized by reason of the fact that a critical balance must be maintained between the elements which promote ferrite and the elements which promote austenite. By assigning a weighted factor corresponding to each element's relative strength in this respect, and by incorporating these factors into a ratio of austenite-forming elements to ferrite-forming elements, a numerical index is obtained which represents the chemistry of each heat and the composition limits within which each heat must fall in order to obtain the optimum combination of good hot workability and excellent machinability. This numerical index, then, must fall within certain given limits, as will be more clearly set forth hereinafter. Based on production experience, it has been found that the ratio of the austenite formers to ferrite formers can be expressed as:

$$\gamma/\alpha = \frac{40(\% C + \% N) + 3(\% Ni) + 2(\% Mn)}{(\% Cr) + 5.2(\% Si)}$$

Using the foregoing equation, it has been found that from the aspect of total chemistry alone, an alloy having a numerical index, as computed by the above formula, which falls within the range between 1.83 and 2.67 will possess an outstanding combination of hot workability and machinability. However, even though an alloy may have a numerical index within the given range, certain other considerations are also significant.

It has been found that the addition of sulfur to the alloy enhances its machinability. However, the range must be critically restricted in order to prevent hot workability difficulties from occurring to the alloy. Our experience has dictated that the sulfur must be present within the range between 0.025% and 0.055% in order to effect the improvement in machinability without causing any hot working difficulties. Significant improvement of machinability has not been found in the subject alloy where the sulfur content is increased to above 0.055%. Accordingly, there is no advantage which exists to warrant running the risk of hot workability difficulties with the use of higher sulfur contents.

In addition to the foregoing, it has also been found that the nitrogen content is also highly critical within the range stated in Table I. Nitrogen, being an interstitial hardener, has a great influence on the strain hardening rate of the alloy. Moreover, the nitrogen content also provides additional strength and materially contributes to the austenitic stability of the alloy. The nitrogen content must be above 0.18% in order to maintain the requisite degree of strength and hardness, together with sufficient austenitic stability, whereas if the nitrogen content is increased to above about 0.28%, the alloy strain-hardens quite rapidly with the result that the machinability of the alloy is adversely affected.

Each of the critical factors, that is, the austenite to ferrite balance as expressed by the numerical index, the sulfur content and the nitrogen content, are quite interrelated. Consequently, it is necessary to perform some test in which all the variables are eliminated, except the differences in the composition of the material tested. The subject test, which meets these conditions and which has been found to be most practical in evaluating the comparative machinability of these alloys, is a single point lathe turning test. This test was performed on a 16 x 30 American Pacemaker lathe equipped with a variable speed drive to provide constant speed control. A single point C-6 carbide tool was used to machine 1-inch diameter hot rolled bar stock in both the solution treated and the solution treated plus aged condition. A constant speed

of 100 feet per minute, feed at the rate of 0.009 inch per revolution, and depth of cut of 0.050 inch were maintained for all tests. The tool angles were also maintained constant as follows:

Back rake—5°, negative  
Side rake—5°, negative  
Side cutting edge angle, 15°  
End cutting edge angle, 15°  
Relief, 5°  
Nose radius,  $\frac{1}{32}$ "

The tests were run without a cutting fluid, and the relative machinability of the alloy from each heat was ascertained through a measurement of the time required to produce a predetermined amount of tool wear. Thus the combined effects of the aforementioned factors of the ratio of the austenite formers to ferrite formers as expressed by the numerical index, the sulfur content and the nitrogen content, can be illustrated by correlation with the relative machinability ratings. These ratings are graphically illustrated by the plots of tool life in minutes versus the wear of the tool land in thousandths of an inch. In comparing the curves set forth in FIGS. 1 and 2, the optimum machining curve possesses a high slope and is located at the left-most side of the plot. Thus the machinability of the alloy diminishes as the curve shifts from left to right on the plot, and as the slope decreases. As illustrated in FIG. 1, Heat No. 40838 exhibits the best machinability of all the heats reported since it has the highest slope and is located at the left-most side of the plot. It is significant to point out that the gamma to alpha ratio was ideal, being 2.29, the nitrogen content was at the high end of the analysis range, and the sulfur content was at about the high end of the range. By thus maintaining the nitrogen and sulfur contents within the ranges specified with the proper numerical index, the alloy exhibits excellent machinability.

While Heat No. 04732 appeared to be the next most machinable heat, it was far inferior to Heat No. 40838. Comparison of the chemical analyses reveals that while both heats possessed similar sulfur contents, the extremely high nitrogen content of Heat No. 04732, together with its extremely high numerical index (3.25), clearly illustrates the adverse effect of these latter two factors upon the machinability of the alloy.

Continuing the comparison, Heat No. 40839, which exhibits a good initial machinability, clearly illustrates the adverse effect of high nitrogen contents on the machinability of the alloy. Similarly, Heat No. 40802, which has a good numerical index and a nitrogen content within the given range, clearly shows the adverse effect of low sulfur contents. Heat No. 40836 has a high numerical index and a low sulfur content, and consequently exhibits poor machinability.

Reference is now respectfully directed to FIG. 2 which illustrates the relative machinability of some of these steels when they are machined in their solution treated plus aged condition. Once again it is clear that Heat No. 40838 clearly possesses outstanding machinability characteristics when compared with Heat No. 04588, the latter being of the Alloy X analysis. Heat No. 40802 is included for comparison purposes, and clearly illustrates the effect of the low sulfur content where the optimum numerical index and nitrogen contents are present.

From the foregoing it is clear that the alloy of the present invention must be maintained within critical limits of the chemical composition as set forth in Table I. In addition, the chemical composition must be so balanced as to provide the proper austenite to ferrite-forming elements ratio as expressed by the numerical index. In addition, it has been found expedient to maintain a critically narrow range of sulfur, together with a narrow range of nitrogen, in order to maintain the optimum combination of properties. As thus balanced, the alloy of the present invention exhibits excellent hot workability and

machinability, and an acceptable combination of chemical, mechanical and physical properties equivalent to the alloys which are presently being used. By thus maintaining the proper balance of the foregoing factors, there appear to be no special metallurgical skills, processes or equipment which are necessary in order to practice the subject invention.

We claim:

1. An austenitic alloy suitable for use at elevated temperatures in atmospheres containing combustion products of leaded fuels and having a composition within the limits 0.65% and 0.75% carbon, 5.50% and 6.90% manganese, 0.45% and 0.85% silicon, 20.50% and 22.0% chromium, 1.40% and 1.90% nickel, 0.18% and 0.28% nitrogen, 0.025% and 0.055% sulfur and the balance essentially iron with incidental impurities and which is characterized by possessing excellent machinability and hot workability.
2. An austenitic alloy suitable for use at elevated temperatures in atmospheres containing combustion products of leaded fuels and having a composition within the limits 0.68% and 0.73% carbon, 6.00% and 6.50% manganese, 0.60% and 0.70% silicon, 21.00% and 21.50% chromium, 1.60% and 1.75% nickel, 0.20% and 0.25% nitrogen, 0.025% and 0.040% sulfur and the balance essentially iron with incidental impurities, and which is characterized by possessing excellent machinability and hot workability.
3. An austenitic alloy suitable for use at elevated temperatures in atmospheres containing combustion products of leaded fuels and having a composition containing about 0.70% carbon, about 6.25% manganese, about 0.65% silicon, about 21.25% chromium, about 1.7% nickel, about 0.22% nitrogen, 0.035% sulfur and the balance essentially iron with incidental impurities, and which is characterized by possessing excellent machinability and hot workability.
4. An austenitic alloy suitable for use at elevated temperatures and in atmospheres containing combustion products of leaded fuels and which is characterized by exhibiting excellent hot workability and machinability, said alloy having a composition within the limits of 0.65% and 0.75% carbon, 5.50% and 6.90% manganese, 0.45% and 0.85% silicon, 20.50% and 22.0% chromium, 1.40% and 1.90% nickel, 0.18% and 0.28% nitrogen, 0.025% and 0.055% sulfur and the balance essentially iron with incidental impurities, and in which the austenite-forming components and the ferrite-forming components of said alloy are balanced within the relationship:

$$50 \quad \frac{40(\% C + \% N) + 3(\% Ni) + 2(\% Mn)}{(\% Cr) + 5.2(\% Si)} = \frac{\gamma}{\alpha}$$

to provide  $\gamma/\alpha$  index within the range between 1.83 and 2.67.

5. An austenitic alloy suitable for use at elevated temperatures and in atmospheres containing combustion products of leaded fuels and which is characterized by exhibiting excellent hot workability and machinability, said alloy having a composition within the limits of 0.68% and 0.73% carbon, 6.00% and 6.50% manganese, 0.60% and 0.70% silicon, 21.0% and 21.5% chromium, 1.60% and 1.75% nickel, 0.20% and 0.25% nitrogen, 0.025% and 0.040% sulfur and the balance essentially iron with incidental impurities, and in which the austenite-forming components and the ferrite-forming components of said alloy are balanced within the relationship:

$$40(\% C + \% N) + 3(\% Ni) + 2(\% Mn) = \frac{\gamma}{\alpha}$$

$$(\% Cr) + 5.2(\% Si)$$

70 to provide  $\gamma/\alpha$  index within the range between 2.08 and 2.38.

6. Stable austenitic valves and valve components characterized by good resistance to thermal fatigue, hot stretching, thermal shock and corrosion in atmospheres containing combustion products of leaded fuels, and

formed from an alloy consisting essentially of 0.65% to 0.75% carbon, 5.50% to 6.90% manganese, 0.45% to 0.85% silicon, 20.50% to 22.00% chromium, 1.40% to 1.90% nickel, 0.18% to 0.28% nitrogen, 0.025% to 0.055% sulfur and the balance essentially iron with incidental impurities.

7. Stable austenitic valves and valve components characterized by good resistance to thermal fatigue, hot stretching, thermal shock and corrosion in atmospheres containing combustion products of leaded fuels, and formed from an alloy consisting essentially of 0.68% to 0.73% carbon, 6.00% to 6.50% manganese, 0.60% to 0.70% silicon, 21.00% to 21.50% chromium, 1.60% to 1.75% nickel, 0.20% to 0.25% nitrogen, 0.025% to 0.040% sulfur and the balance essentially iron with incidental impurities.

8. An article of manufacture of the class including valves and valve components which are suitable for use in exhaust systems of internal combustion engines, said article exhibiting good strength and hardness at operational temperatures of about 1400° F. and good resistance to corrosion, oxidation, thermal fatigue, hot stretching and thermal shock, said article being formed from a stable, austenitic, age-hardenable alloy which is characterized by exhibiting excellent hot workability and machinability resulting from balancing the composition within the range between 0.65% and 0.75% carbon, 5.50% and 6.90% manganese, 0.45% and 0.85% silicon, 20.50% and 22.00% chromium, 1.40% and 1.90% nickel, 0.18% and 0.28% nitrogen, 0.025% and 0.050% sulfur and the balance essentially iron with incidental impurities, to provide a numerical index within the range between 1.83 and 2.67 of the austenite-forming components ( $\gamma$ ) to ferrite-forming components ( $\alpha$ ) as expressed by the relationship:

$$\frac{40(\% \text{ C} + \% \text{ N}) + 3(\% \text{ Ni}) + 2(\% \text{ Mn})}{(\% \text{ Cr}) + 5.2(\% \text{ Si})}$$

$$= \frac{\gamma}{\alpha} = 1.83 \text{ to } 2.67$$

9. An article of manufacture of the class including valves and valve components which are suitable for use in exhaust systems of internal combustion engines, said article exhibiting good strength and hardness at operational temperatures of about 1400° F. and good resistance to corrosion, oxidation, thermal fatigue, hot stretching and thermal shock, said article being formed from a stable, austenitic, age-hardenable alloy which is characterized by exhibiting excellent hot workability and machinability resulting from balancing the composition within the range between 0.68% and 0.73% carbon, 6.00% and 6.50% manganese, 0.60% and 0.70% silicon, 21.00% and 21.50% chromium, 1.60% and 1.75% nickel, 0.20% and 0.25% nitrogen, 0.025% and 0.040% sulfur and the balance essentially iron with incidental impurities, to provide a numerical index within the range between 2.08 and 2.38 of the austenite-forming components ( $\gamma$ ) to ferrite-forming components ( $\alpha$ ) as expressed by the relationship:

$$\frac{40(\% \text{ C} + \% \text{ N}) + 3(\% \text{ Ni}) + 2(\% \text{ Mn})}{(\% \text{ Cr}) + 5.2(\% \text{ Si})}$$

$$= \frac{\gamma}{\alpha} = 2.08 \text{ to } 2.38$$

10. Valves and valve components formed from a stable, austenitic alloy which possesses a composition within the limits between 0.65% and 0.75% carbon, 5.50% and 6.90% manganese, 0.45% and 0.85% silicon, 20.50% and 22.00% chromium, 1.40% and 1.90% nickel, 0.18% and 0.28% nitrogen, 0.025% and 0.055% sulfur and the balance essentially iron with incidental impurities, and which is characterized by exhibiting a minimum hardness of 38 R<sub>c</sub> after forming the valves or valve components by hot working followed by an aging heat treatment at a temperature within the range between 1400° F. and 1700° F. for a time period of up to about 8 hours.

11. Valves and valve components formed from a stable, austenitic alloy having a composition within the limits between 0.65% and 0.75% carbon, 5.50% and 6.90% manganese, 0.45% and 0.85% silicon, 20.50% and 22.00% chromium, 1.40% and 1.90% nickel, 0.18% and 0.28% nitrogen, 0.025% and 0.055% sulfur and the balance essentially iron with incidental impurities, and which is characterized by exhibiting a minimum hardness of 34 R<sub>c</sub> after forming the valves or valve components by hot working followed by a solution heat treatment of the valves and valve components at a temperature within the range between 2100° F. and 2200° F.

20 25 for a time period of from 15 minutes to about 4 hours, quenching and thereafter aging at a temperature within the range between 1400° F. and 1700° F. for a time period ranging between 4 hours and 24 hours.

12. Valve and valve components formed from a stable austenitic alloy which possesses a composition within the limits between 0.65% and 0.75% carbon, 5.50% and 6.90% manganese, 0.45% and 0.85% silicon, 20.50% and 22.00% chromium, 1.40% and 1.90% nickel, 0.18% and 0.28% nitrogen, 0.025% and 0.055% sulfur and the balance essentially iron with incidental impurities, and which is characterized by good creep rupture properties, and hardness without any adverse effect on the machinability after forming the valves by hot working followed by a solution heat treatment at a temperature within the range between 1950° F. and 2050° F. for a time period of up to one hour followed by a quench.

13. Valve and valve components formed from a stable austenitic alloy which possesses a composition within the limits between 0.65% and 0.75% carbon, 5.50% and 6.90% manganese, 0.45% and 0.85% silicon, 20.50% and 22.00% chromium, 1.40% and 1.90% nickel, 0.18% and 0.28% nitrogen, 0.025% and 0.055% sulfur and the balance essentially iron with incidental impurities, and which is characterized by being suitable for use in an internal combustion engine without prior heat treatment after forming the valves by hot working followed by a machining operation where necessary.

#### References Cited in the file of this patent

#### UNITED STATES PATENTS

2,380,821 Breeler et al. ----- July 31, 1945

#### FOREIGN PATENTS

481,629 Canada ----- Mar. 11, 1952